

Patented June 28, 1949

2,474,293

UNITED STATES PATENT OFFICE

2,474,293

1-NAPHTHOL-2-CARBOXYLIC ACID AMIDE  
COUPLERS FOR COLOR PHOTOGRAPHY

Arnold Weissberger, Ilmari F. Salminen, and Paul W. Vittum, Rochester, N. Y., assignors to Eastman Kodak Company, Rochester, N. Y., a corporation of New Jersey

No Drawing. Application September 10, 1947,  
Serial No. 773,290

7 Claims. (Cl. 95—6)

1

This invention relates to photography and particularly to compounds which form dye by coupling with the developing agent to produce colored images.

It is known that colored photographic images may be formed by using a developer which produces a colored compound on development. The colored compound thus formed is deposited adjacent the silver grains of the silver image during development. It is also known that a colored image may be formed by adding to certain developing solutions or by incorporating in the silver halide emulsion a compound which couples during development with the oxidation product of the developing agent and forms a colored compound which is likewise deposited adjacent the silver grains of the silver image during development. Such a compound which is employed in conjunction with a developing agent for the silver and which couples with the oxidation product of the developing agent during development is referred to herein as a coupling compound or coupler.

The present invention concerns new and improved color-forming couplers for use with a primary aromatic amino developing agent and also includes a new and improved color development process which consists in developing a reducible silver salt image in a photographic emulsion with the aid of a primary aromatic amino developer and in the presence of a coupler as hereinafter defined. The invention also includes photographic sensitive elements having such coupler in one or more of the sensitive emulsion layers.

We have found that compounds of the following structure are valuable couplers for color photography and produce blue-green images of high purity and stability on photographic development.



where Z is hydrogen or a chlorine atom, R and R' represent the same or different alkyl radicals of from 1 to 5 carbon atoms, that is, methyl, ethyl, propyl, butyl or amyl, n is an integer of from 2 to 4 and y is 0 or 1.

The following compounds illustrate our invention:



1-hydroxy-2-[δ-(2',4'-di-tert. amylphenoxy)-n-butyl]-naphthamide

2



1-hydroxy-2-[δ-(2',4'-di-tert. amylphenoxy)-n-butyl]-4-chloro-naphthamide



1-hydroxy-2-[β-(2',4'-di-tert. amylphenoxy)-ethyl]-naphthamide



1-hydroxy-2-[β-(2',4'-di-tert. amylphenoxy)-ethyl]-4-chloro-naphthamide



1-hydroxy-2-[δ-(2',4'-di-tert. amylphenoxy)-propyl]-naphthamide



1-hydroxy-2-[δ-(2'-n-butyl-4'-tert. amylphenoxy)-n-butyl]-naphthamide



1-hydroxy-2-[δ-(p-tert. amylphenoxy)-n-butyl]-naphthamide



1-hydroxy-2-[β-(2',4'-tert. diethylphenoxy)-acetamido]-naphthamide



These couplers contain a coupling function which in this case is a phenolic hydroxyl group. Coupling is believed to occur in a position para to the hydroxyl group of the naphthol radical and in case a chlorine atom is present in this position, it is split off during the coupling.

Our compounds may be prepared by reacting a suitable amine with 1-naphthol-2-carboxylic acid chloride or 1-naphthol-2-carboxylic acid phenyl ester (Ber., 20, 2700) or the 4-chloro derivative of either of these compounds. For example, compounds 1 and 2 are prepared as follows:

Commercial 2,4-tert.-diamylphenol and  $\gamma$ -chlorobutyronitrile are condensed in the presence of alkali. The resultant  $\gamma$ -2,4-tert.-diamylphenoxybutyronitrile is reduced to  $\delta$ -2,4-tert.-diamylphenoxybutylamine and the amine condensed with an equivalent amount of 1-naphthol-2-carboxylic acid phenyl ester to give compound 1, or

 $\beta$ -2,4-TERT.-DIAMYLPHENOXYPROPIONITRILE

In a 200-cc. round-bottomed flask was placed 47 g. (0.2 mole) of diamylphenol (alkali-washed) and 32 g. of redistilled acrylonitrile. The temperature rose from 24 to 26.5°. To this solution was added 4 cc. of trimethylbenzyl ammonium hydroxide solution. The quaternary hydroxide solution failed to mix with the ether until 25 cc. of dioxane had been added also.

The solution stood in a stoppered flask for 3 days, after which it was removed, drowned in 400 cc. of water, extracted with three 200-cc. portions of ether, the emulsion being broken with 4 g. of barium chloride. The ether solution was washed with three 200-cc. portions of water, dried over sodium or magnesium sulfate, filtered, and concentrated by distillation on a steam bath.

The residual liquid was distilled in vacuo at 136-142°/1 mm. Yield = 47 g. (82%).

## Molecular weights

|                                               |       |     |
|-----------------------------------------------|-------|-----|
| Diamylphenol                                  | ----- | 234 |
| Acrylonitrile                                 | ----- | 53  |
| $\beta$ -2,4-tert.-diamylphenoxypropionitrile | ----- | 287 |

 $\gamma$ -(2,4-TERT.-DIAMYLPHENOXYPROPYL)-AMINE

with the 4-chloro derivative to give compound 2. Compounds 3 and 4 are prepared as follows:

Ethylenimine and 2,4-tert.-diamylphenol are condensed hot to give  $\beta$ -2,4-tert.-diamylphenoxyethylamine. The amine is condensed with an equivalent amount of 1-naphthol-2-carboxylic acid phenyl ester to give compound 3, or with the 4-chloro derivative to give compound 4.

Compound 5 is prepared as follows:

2,4-tert.-diamylphenol is condensed with acrylonitrile in the presence of alkali, giving  $\beta$ -2,4-tert.-diamylphenoxypropionitrile. The nitrile is reduced catalytically to the amine, which is condensed with 1-naphthol-2-carboxylic acid phenyl ester to yield compound 5.

Compounds 6 and 7 are prepared like compounds 1 and 2, with the use of commercial amyloxyphenol for 6 and p-tert.-amylphenol for 7.

Compound 8 is prepared as follows:

1-naphthol-2-carboxylic acid phenyl ester is condensed with ethylene diamine, giving 1-hydroxy-2- $\beta$ -aminoethyl naphthamide. The amino-naphthamide is condensed with 2,4-tert.-diamylphenoxyacetyl chloride to give compound 8.

Compound 9 is prepared like compound 8, with the use of 4-chloro-1-naphthol-2-carboxylic acid phenyl ester.

Compound 10 is prepared like compound 8, with the use of tetramethylene diamine.

The detailed preparation of compound 5, for example, is as follows:

45 In the low-pressure shaker was placed 40 g. (0.1 mole) of  $\beta$ -2,4-diamylphenoxypropionitrile, 150 cc. of white label methanol and Raney nickel which had been washed four times with distilled water, followed by four times with methanol. The mixture was heated with steam and reduced while shaking. Reduction was rapid, the hydrogen pressure dropping from 59 to 35 lbs. in 1 hr. Only 1 lb. more was absorbed during an additional half hour.

50 The mixture was filtered from Raney nickel. The filtrate was concentrated by distillation up to an oil bath temperature of 125°.

The 38.6 g. of residual liquid was distilled in vacuo, fractions being collected as follows:

|                             |         |              |        |
|-----------------------------|---------|--------------|--------|
| No. 1, B. P. 113-130°/1 mm. | 6.0 g.  | $n_{D}^{20}$ | 1.5092 |
| No. 2, B. P. 131-139°/1 mm. | 25.3 g. | $n_{D}^{20}$ | 1.5090 |
| No. 3, B. P. 140-150°/1 mm. | 3.8 g.  | $n_{D}^{20}$ | 1.5058 |
| No. 4, residue              | 3.2 g.  | $n_{D}^{20}$ | 1.5112 |

60 Fraction No. 2 was the product. Yield = 62%. Even when reduced according to these directions some cleavage occurs as can be shown by collecting or smelling the volatile low molecular weight amine.

## Molecular weights

65  $\beta$ -2,4-tert.-diamylphenoxypropionitrile ----- 287

75  $\gamma$ -(2,4-tert.-diamylphenoxypropyl)-amine - 291

5

1-HYDROXY-2-( $\gamma$ -2',4'-TERT.-DIAMYLPHENOXY-  
PROPYL)-NAPHTHAMIDE

In a Claisen flask, set up for vacuum distillation, was placed 6.0 g. (0.02 mole) of  $\gamma$ -(2',4'-tert-diamylphenoxypropyl)-amine (fraction No. 2) and 5.3 g. (0.02 mole) of phenyl 1-hydroxy-2-naphthoate. The flask was immersed in a pre-heated oil bath at 145-150° for one-half hour. Vacuum was applied to the amber melt and phenol removed by distillation. After 5 mins. 1.65 g. of distillate had been collected. Following another 15 mins., the temperature of the bath having risen to 160°, 2.35 g. of distillate had been collected. The cooled reaction mixture was diluted with 10 cc. of petroleum ether and seeded with product from a previous preparation. Some solid appeared. The mixture stood overnight in an open flask, the solvent evaporating and leaving behind a pale yellow semi-crystalline residue. This residue was stirred for 1 hr. with 100 cc. of petroleum ether, cooled in an ice bath and filtered at 5° C. The solid was washed on the funnel with three 5-cc. portions of cold petroleum ether. Yield: 4.5 g. (50%); M. P. 91-93°. Recrystallization of the product from hexane or ligroin gave better looking crystals but did not raise the melting point.

## Molecular weights

|                                                                          |     |
|--------------------------------------------------------------------------|-----|
| $\gamma$ -(2,4-tert-diamylphenoxypropyl)-amine                           | 291 |
| Phenyl 1-hydroxy-2-naphthoate                                            | 264 |
| 1-hydroxy-2-( $\gamma$ -2',4'-tert-diamylphenoxy-<br>propyl)-naphthamide | 461 |

Our compounds may be used either in the developing solution or in the sensitive emulsion layer. Where the compounds are of suitable molecular size as in the case of compounds 1 to 10, they may be incorporated in the sensitive emulsion layer or in one of the layers of a multi-layer coating. When incorporated in a photographic emulsion layer, we prefer to incorporate the couplers in the manner described in Mannes and Godowsky U. S. Patent 2,304,940 or Jelley and Vittum U. S. Patent 2,322,027.

The aromatic amino developing agents used with the coupler compounds of our invention include the p-phenylene diamine type or their derivatives formed by substitution in one of the amino groups or in the ring such as the alkyl phenylene diamine and alkyl toluene diamines. These compounds are usually used in the salt form such as the hydrochloride or the sulfate which is more stable than the amines themselves. Suitable compounds are diethyl p-phenylene diamine hydrochloride, dimethyl-p-phenylene diamine hydrochloride and 2-amino-5-diethylamino toluene hydrochloride. Developing agents containing heterocyclic systems as described in U. S. Patent 2,196,739 are also suitable. The p-amino phenols and their substitution products may also be used where the amino group is unsubstituted. All of these compounds have an unsubstituted amino group which enables the oxidation product of the developer to couple with the color-forming compounds to form a dye image.

6

The following example illustrates a developing solution which may be used with the compounds of our invention where the compounds are incorporated in the emulsion layer.

|                               | Grams |
|-------------------------------|-------|
| p-Aminodiethylaniline sulfate | 2     |
| Sodium sulfite (anhydrous)    | 5     |
| Sodium carbonate (anhydrous)  | 20    |
| Potassium bromide             | 2     |
| Water to one liter.           |       |

Our development process may be employed for the production of colored photographic images in layers of gelatin or other carrier for the silver halide such as collodion, organic esters of cellulose or synthetic resins. The support for the emulsion may be a transparent material such as glass, cellulose ester or a non-transparent reflecting material such as paper or an opaque cellulose ester. The emulsion may be coated as a single layer on the support or as one of a series of superposed layers on one or both sides of the support. The superposed layer may be differentially sensitized to record natural color photographic images in the well known manner.

The examples and compounds set forth in the present specification are illustrative only and it is to be understood that our invention is to be taken as limited only by the scope of the appended claims.

We claim:

1. A photographic emulsion for forming colored images comprising a silver halide emulsion having incorporated therein a coupler compound having the formula:



where Z is selected from the class consisting of hydrogen and chlorine, R and R' are alkyl groups of from 1 to 5 carbon atoms, n is an integer from 2 to 4, and y is selected from the class consisting of 0 and 1.

2. A photographic emulsion for forming colored images comprising a silver halide emulsion having incorporated therein a coupler compound having the formula:



where Z is selected from the class consisting of hydrogen and chlorine, R and R' are alkyl groups of from 1 to 5 carbon atoms and n is an integer from 2 to 4.

3. A photographic emulsion for forming colored images comprising a silver halide emulsion having incorporated therein a coupler compound having the formula:



4. A light-sensitive emulsion for producing a colored image comprising a gelatino silver halide emulsion containing finely divided liquid particles

of a mixture of a coupler compound having the formula:



where Z is selected from the class consisting of hydrogen and chlorine, R and R' are alkyl groups of from 1 to 5 carbon atoms, n is an integer from 2 to 4, and y is selected from the class consisting of 0 and 1 and a substantially water-insoluble low molecular weight organic crystalloidal material having a boiling point above about 175° C. 10

5. The method of producing a colored photographic image in a silver halide emulsion layer which comprises exposing said layer and developing it with a primary aromatic amino developing agent in the presence of a coupler compound having the formula:



where Z is selected from the class consisting of hydrogen and chlorine, R and R' are alkyl groups of from 1 to 5 carbon atoms, n is an integer from 2 to 4, and y is selected from the class consisting of 0 and 1. 30

6. The method of producing a colored photo-

graphic image in a silver halide emulsion layer which comprises exposing said layer and developing it with a primary aromatic amino developing agent in the presence of a coupler compound having the formula:



where Z is selected from the class consisting of hydrogen and chlorine, R and R' are alkyl groups of from 1 to 5 carbon atoms and n is an integer from 2 to 4. 15

7. The method of producing a colored photographic image in a silver halide emulsion layer which comprises exposing said layer and developing it with a primary aromatic amino developing agent in the presence of a coupler compound having the formula:



ARNOLD WEISSBERGER.  
ILMARI F. SALMINEN.  
PAUL W. VITTM.

No references cited.

**Certificate of Correction**

June 28, 1949.

Patent No. 2,474,293.

ARNOLD WEISSBERGER ET AL.

It is hereby certified that errors appear in the printed specification of the above numbered patent requiring correction as follows:

Column 3, Compound 9, for that portion of the structural formula reading



Compound 10, same column, line 17, for that portion of the name under the structural formula reading "n-butyl naphthamide" read *n-butyl}naphthamide*; and that the said Letters Patent should be read with these corrections therein that the same may conform to the record of the case in the Patent Office.

Signed and sealed this 22nd day of November, A. D. 1949.

[~~SEAL~~]

THOMAS F. MURPHY,  
*Assistant Commissioner of Patents.*